

## UNITED STATES PATENT OFFICE

2,253,641

## TREATMENT OF TEXTILE AND OTHER MATERIALS

Robert Wighton Moncrieff and Albert William Mortimer Cooke, Spondon, near Derby, England, assignors to Celanese Corporation of America, a corporation of Delaware

No Drawing. Application June 30, 1938, Serial No. 216,750. In Great Britain August 13, 1937.

2 Claims. (Cl. 8—35)

This invention relates to the treatment of textile and other materials and particularly to the treatment of textile and other materials having a basis of organic esters of cellulose.

Materials having a basis of organic esters of cellulose have not, in general, any affinity for the dyestuffs usually employed in dyeing cotton but, as is well known, such materials acquire an affinity for cotton dyestuffs if they are subjected to saponification prior to the dyeing treatment.

It has now been discovered that colourations which are particularly fast to scouring treatments may be obtained by applying to textile and other materials having a basis of organic esters of cellulose saponifying media containing salts of acid esters of leuco vat dyestuffs, and thereafter effecting oxidation of the leuco vat dyestuffs on the materials.

Preferably the salt employed is a salt of a sulphuric ester of a leuco vat dyestuff though salts of esters formed from other polybasic acids may also be employed, e. g. salts of phosphoric esters. In general, the salts employed will be salts of inorganic bases, e. g. sodium salts or potassium salts, though salts of organic bases may also be employed.

The saponifying media employed may contain any suitable saponifying agents for cellulose esters. Preferably the saponifying agent employed is an organic base, e. g. methylamine, ethylene diamine, benzylamine, cyclohexylamine and guanidine. However, inorganic saponifying agents may be employed, e. g. caustic soda, caustic potash and alkali carbonates. Mixtures of saponifying agents may be employed if desired. Preferably the saponifying agents are employed in aqueous solution. A very suitable saponifying medium for the purpose of the present invention is a 10% aqueous solution of methylamine.

The treatment with the saponifying medium containing the leuco vat dyestuff derivative referred to above may be effected under conditions wherein only partial saponification of the cellulose ester materials takes place, or may be effected so that the cellulose ester materials are completely saponified.

The salt of an acid ester of a leuco vat dyestuff employed according to the invention may be derived from a vat dyestuff of the indigoid series or of the anthraquinone series. Of particular value are dyestuffs of the types marketed under the trade name "Indigosol" and under the registered trade-mark "Soledon." Mixtures of salts of acid esters of leuco vat dyestuffs may be employed if desired.

The saponifying medium containing the leuco vat dyestuff derivative may be applied to textile materials which are in fabric form or in the form of filaments or the like. Thus, textile materials, e. g. in the form of fabrics or hanks of yarns, may be immersed and allowed to stand in the vessel containing the saponifying medium. Or again, yarn wound on perforated bobbins may be treated with the saponifying medium by passing the saponifying medium from the outside to the inside of the bobbins, and vice versa repeatedly.

The oxidation of the leuco vat dyestuff derivative on the materials after the treatment with the saponifying medium during which such leuco vat dyestuff derivative has been applied to the materials may be effected by any suitable means. A convenient method is to treat the materials with a dilute solution of an oxidising agent such as nitrous acid.

The following example illustrates the invention but is not to be regarded as limiting it in any way:

## Example

A 10% aqueous solution of methylamine containing 20 grams of Soledon Jade Green XS (which is a 50% paste) per litre and 14—15 grams of Indigosol Olive Green 1B powder per litre is passed alternately from the outside to the inside and vice versa of perforated bobbins of stretched cellulose acetate yarn, and this treatment is continued for a period of 5 hours at 25° C. The bobbins are then well washed with cold water and a dilute aqueous solution of nitrous acid is passed alternately from the outside to the inside and vice versa for a period of  $\frac{1}{2}$  an hour, during which time the temperature of such solution is gradually raised to 60° C. The yarn on the bobbin was then found to be dyed a full shade of green which was particularly fast to scouring treatments.

A similar treatment using, instead of the dyestuffs specified above, 4 grams per litre of Soledon Blue 4 BCS powder was found to yield a blue colouration also of excellent fastness to scouring.

The depth of colour obtained can be somewhat increased by the addition of sodium chloride to the solution of the saponifying agent and leuco dyestuff derivative.

The invention is of special importance in connection with the treatment of textile and other materials having a basis of cellulose acetate but it may also be applied to the treatment of textile and other materials having a basis of other cellulose esters, e. g. cellulose formate, cellulose propionate, cellulose butyrate and mixed esters and

ether-esters of cellulose as, for example cellulose acetate-propionate, cellulose acetate-butyrate and ethyl cellulose acetate. The textile materials treated may, if desired, be subjected to various other treatments prior to their saponification and colouration by the process of the present invention. Thus, for example, in order to obtain products having a high tensile strength, it is desirable that the textile materials in yarn form should be subjected to a stretching process while in the softened condition prior to their treatment according to the present invention.

The invention has been described above with particular reference to the colouration of textile materials but it may also be applied to the colouration of other materials having a basis of organic esters of cellulose, e. g. films, foils, sheets and moulded articles.

Having described our invention what we desire to secure by Letters Patent is:

1. Process for the coloration of textile materials having a basis of organic esters of cellulose, which comprises subjecting the materials to the action of an aqueous bath containing sodium chloride, 10% of methylamine and a salt of a sulphuric acid ester of a leuco vat dyestuff, and thereafter converting said salt to the parent vat dyestuff on the materials.

2. Process for the coloration of textile materials having a basis of cellulose acetate, which comprises subjecting the materials to the action of an aqueous bath containing sodium chloride, 10% of methylamine and a salt of a sulphuric acid ester of a leuco vat dyestuff, and thereafter converting said salt to the parent vat dyestuff on the materials.

ROBERT WIGHTON MONCRIEFF.  
ALBERT WILLIAM MORTIMER COOKE.